

Sept. 30, 1930.

J. BRUIJNES ET AL

1,777,253

OXIDE CATHODE

Filed Feb. 25, 1927



INVENTORS

Johannes Bruijnes  
Jacob vander Hoeven  
EKKO Oosterhuis

Langmuir, Percy, Ward & Langmuir <sup>by</sup> Attys.

## UNITED STATES PATENT OFFICE

JOHANNES BRUIJNES, JACOB VAN DER HOEVEN, AND EKKO OOSTERHUIS, OF EINDHOVEN, NETHERLANDS, ASSIGNEES TO N. V. PHILIPS' GLOEILAMPEN-FABRIEKEN, OF EINDHOVEN, NETHERLANDS, A LIMITED LIABILITY COMPANY

## OXIDE CATHODE

Application filed February 25, 1927, Serial No. 171,051, and in the Netherlands April 6, 1928.

This invention is concerned with an incandescent cathode for electric discharge tubes of the type in which a substance of high emitting capacity such, for example, as the oxide of one or more alkaline earth metals is applied to a core which itself takes no part in the emission.

An object of the invention is to provide an incandescent cathode having a long life. 10 Another object of the invention is to increase the current of electrons emitted by an incandescent cathode per unit of length.

Other objects will appear from the following description of the invention, made 15 with reference to the accompanying drawing which shows an embodiment of an incandescent cathode according to the invention.

The incandescent cathode according to the invention has a core of highly refractory 20 metal, preferably a poor conductor of heat, on which is helically wound another metal wire having applied to it a substance of high emitting capacity.

It is preferable that an element selected 25 from the left hand members of Group VI of the periodic system between atomic numbers 41 and 75 for example, in the form of a wire, be used for the core, a metal wire which is preferably coated with alkaline earth oxide, 30 being then wound on the said core so as to be in electrical contact therewith. Preferably platinum or a platinum alloy is used for the winding wire. In the drawing a stretched core wire 1 made, for example, of tungsten 35 or molybdenum has helically wound on it a wire 2. The turns of the latter wire may be adjacent each other, as shown in the drawing but also they may be wound quite well so as to be slightly spaced apart, if this should be 40 desirable for any reason, for example, in view of the steepness of the discharge tube for which the cathode is intended.

The wire 2 which is preferably made of platinum or a platinum alloy (for example 45 platinum-rhodium) is coated with a film of a substance of high emission capacity, for example barium oxide. This oxide may be applied to the wire 2 in one of the ways known for this purpose, for example, by first coating the wire with copper, oxidizing the cop-

per and precipitating metallic barium on the copper oxide. The barium reduces the copper in the presence of heat and by additional heat the reduced copper is evaporated, leaving barium oxide on the wire. The wire 55 2 may be coated with copper and oxidized before it is wound on the core 1 and only then the barium may be precipitated.

In the example illustrated the core wire 1 extends on both sides outside the ends of the wire spiral 2 and the ends of the wire 2 are secured to the said protruding ends of the core wire 1, which are finally attached to leads 3 and 4 which serve to supply the current and which are secured in a known manner to the glass pinch of a lamp foot. 60 65

However, it is also possible to make the core wire with the emission wire wound on it in continuous lengths, to divide it into portions of the required length and to set the 70 said portions tightly between the leads. The example illustrated has, however, the advantage that the temperature will be substantially uniform all along the emitting surface by reason of the comparatively poor 75 conduction of heat on the part of the free ends of the core wire 1. When the incandescent cathode is used in a discharge tube comprising one or more auxiliary electrodes, the so-called steepness is thus favourably influenced. 80 85

What we claim is:

1. An incandescent cathode comprising a core of highly refractory metal, a metal wire helically wound on the said core so as to be 90 in electrical contact therewith, and a substance of high electron emitting capacity applied to said wire. 95

2. An incandescent cathode, comprising a core consisting of at least one of the metals tungsten and molybdenum, a metal wire helically wound on the core so as to be in electrical contact therewith, and a substance of high electron emitting capacity comprising an alkaline earth oxide applied to said wire. 100

3. An incandescent cathode comprising a core consisting of at least one of the metals tungsten and molybdenum, a metal wire comprising platinum helically wound on the core so as to be in electrical contact therewith, 105

and a substance of high electron emitting capacity comprising an alkaline earth oxide applied to said wire.

4. An incandescent cathode comprising a core consisting of at least one of the metals tungsten and molybdenum, a platinum wire helically wound on the core so as to be in electrical contact therewith, and a substance of high electron emitting capacity comprising an alkaline earth oxide applied to said wire.

5. An incandescent cathode, comprising a core consisting of an element of the left hand members of Group VI of the periodic system between atomic numbers 41 and 75, a metal wire helically wound on the core so as to be in electrical contact therewith, and a substance of high electron emitting capacity comprising an alkaline earth oxide applied to said wire.

6. An incandescent cathode comprising a core consisting of an element of the left hand members of Group VI of the periodic system between atomic numbers 41 and 75, a metal wire comprising platinum helically wound on the core so as to be in electrical contact therewith, and a substance of high electron emitting capacity comprising an alkaline earth oxide applied to said wire.

7. An incandescent cathode comprising a core consisting of an element of the left hand members of Group VI of the periodic system between atomic numbers 41 and 75, a platinum wire helically wound on the core so as to be in electrical contact therewith, and a substance of high electron emitting capacity comprising an alkaline earth oxide applied to said wire.

In testimony whereof we affix our signatures, at the city of Eindhoven, this 4th day February, A. D. 1927.

JOHANNES BRUIJNES.  
JACOB VAN DER HOEVEN.  
EKKO OOSTERHUIS.

45

#### DISCLAIMER

1,777,253.—*Johannes Bruijnes, Jacob van der Hoeven, and Ekko Oosterhuis, Eindhoven, Netherlands. OXIDE CATHODE.* Patent dated September 30, 1930. Disclaimer filed July 13, 1932, by the assignee, *N. V. Philips' Gloeilampenfabrieken*.

Hereby enters this disclaimer to those parts of certain claims in said specification which are in the following words, to wit:

In the claims, where the language "a wire helically wound on the core so as to be in electrical contact therewith" is employed, your petitioner disclaims the use of any construction other than where the wire is shorted directly on the core throughout the length of the wire.

[*Official Gazette August 9, 1932.*]

and a substance of high electron emitting capacity comprising an alkaline earth oxide applied to said wire.

4. An incandescent cathode comprising a core consisting of at least one of the metals tungsten and molybdenum, a platinum wire helically wound on the core so as to be in electrical contact therewith, and a substance of high electron emitting capacity comprising an alkaline earth oxide applied to said wire.

5. An incandescent cathode, comprising a core consisting of an element of the left hand members of Group VI of the periodic system between atomic numbers 41 and 75, a metal wire helically wound on the core so as to be in electrical contact therewith, and a substance of high electron emitting capacity comprising an alkaline earth oxide applied to said wire.

6. An incandescent cathode comprising a core consisting of an element of the left hand members of Group VI of the periodic system between atomic numbers 41 and 75, a metal wire comprising platinum helically wound on the core so as to be in electrical contact therewith, and a substance of high electron emitting capacity comprising an alkaline earth oxide applied to said wire.

7. An incandescent cathode comprising a core consisting of an element of the left hand members of Group VI of the periodic system between atomic numbers 41 and 75, a platinum wire helically wound on the core so as to be in electrical contact therewith, and a substance of high electron emitting capacity comprising an alkaline earth oxide applied to said wire.

In testimony whereof we affix our signatures, at the city of Eindhoven, this 4th day February, A. D. 1927.

JOHANNES BRUIJNES.  
JACOB VAN DER HOEVEN.  
EKKO OOSTERHUIS.

45

#### DISCLAIMER

1,777,253.—*Johannes Bruijnes, Jacob van der Hoeven, and Ekko Oosterhuis, Eindhoven, Netherlands. OXIDE CATHODE.* Patent dated September 30, 1930. Disclaimer filed July 13, 1932, by the assignee, *N. V. Philips' Gloeilampenfabrieken*.

Hereby enters this disclaimer to those parts of certain claims in said specification which are in the following words, to wit:

In the claims, where the language "a wire helically wound on the core so as to be in electrical contact therewith" is employed, your petitioner disclaims the use of any construction other than where the wire is shorted directly on the core throughout the length of the wire.

[*Official Gazette August 9, 1932.*]